

# United States Patent Office

2,849,337

Patented Aug. 26, 1958

1

2,849,337

## METAL COATING BATHS

John W. Robinson, Brecksville, Ohio, assignor to the United States of America as represented by the United States Atomic Energy Commission

No Drawing. Application November 28, 1945  
Serial No. 631,482

1 Claim. (Cl. 117—114)

The present invention relates to the maintenance of 15 bronze coating baths and is particularly concerned with a method for restoring the effectiveness of bronze coating baths used for coating uranium by hot dip coating processes.

In the application of bronze coatings to uranium by 20 dipping the uranium object to be coated into a molten metal bath, it has been found that after extended use without a flux coating baths of high copper content tend to lose their ability to wet uranium.

An object of the present invention is to restore to 25 bronze coating baths their ability to wet metallic uranium. A further object is to facilitate the maintenance of high-copper bronze baths employed dry for application of hot-dip coatings to uranium.

In accordance with the present invention a bronze bath, 30 which consists predominantly of copper and which has lost its initial ability to wet metallic uranium rapidly, is treated with a small proportion of metallic aluminum. It has been found that this treatment restores to the bronze bath, which consists predominantly of copper and which has lost its initial ability to wet metallic uranium rapidly, is treated with a small proportion of metallic aluminum. It has been found that this treatment restores to the bronze bath its ability to wet the 35 metallic uranium. The aluminum reacts with metals present in the bath to form a hard alloy which can be separated as scum from the bath.

The process is particularly applicable to dry bronze 40 baths of high copper content since baths containing less

than about 50% copper do not become subject to the difficulty encountered with the high-copper baths and the use of flux on bronze baths of high copper content also seems to avoid the difficulty.

### Example

A bronze bath containing 67% by weight copper and 33% by weight tin had been used for some time for the coating of metallic uranium objects. A small metallic 5 uranium rod was dipped in the bath for 1½ minutes while the bath temperature was 830–840° C. Upon removal from the bath the rod was uncoated. 20 grams of 2S metallic aluminum, that is, commercially pure aluminum having a minimum of 99% aluminum, corresponding to  $\frac{1}{30}$  of the weight of the bath, was added to the bath and the resulting hard alloy was removed by skimming. The uranium metal rod was again dipped in the bath for 1½ minutes while the bath temperature was between 830° and 840° C. and upon withdrawal was found to be evenly coated with the bronze coating metal.

A second metallic uranium rod was dipped into the same bath at a temperature between 810° and 790° C. for 45 seconds and upon removal was found to be substantially uniformly coated with the bronze coating metal.

It will be understood that I intend to include variations and modifications of the invention and that the preceding examples are illustrations only and in no wise to be construed as limitations upon the invention, the scope of which is defined in the appended claim, where-

in I claim:

In the process of coating metallic uranium with an alloy of copper and tin by hot dipping the uranium in a bath comprising approximately 67% copper and 33% tin, the method of regenerating a bath which has lost its 35 ability after extended use to wet uranium which comprises adding to the bath metallic aluminum in amount corresponding to  $\frac{1}{30}$  of the weight of the bath.

### References Cited in the file of this patent

#### UNITED STATES PATENTS

|           |          |               |
|-----------|----------|---------------|
| 1,691,207 | Pacz     | Nov. 13, 1928 |
| 2,197,622 | Senzimir | Apr. 16, 1940 |
| 2,307,512 | Kelly    | Jan. 5, 1943  |